

## UNITED STATES PATENT OFFICE

2,001,753

COATED COPPER ARTICLE AND METHOD  
OF MAKING THE SAME

Robert B. Tanner, Highland Park, and John S. Thompson, Detroit, Mich., assignors to Metal Finishing Research Corporation, Detroit, Mich., a corporation of Michigan

No Drawing. Application June 4, 1934,  
Serial No. 728,978

5 Claims. (Cl. 148—6)

This invention has for its object an article having a surface of copper or copper alloy with a paint-holding coating chemically formed thereon, and a method of forming such coating. The object of the invention is to provide articles with surfaces of the kind described which can be finished or decorated with any desired siccative coating and have the finish firmly adhere thereto.

The coating may be produced by a solution of an organic acid of the group consisting of the dicarboxylic and hydroxydicarboxylic acids of the aliphatic series and carboxylic acids, having but one carboxyl group, and sulphonic acids of the aromatic series, and benzene phosphonic acid. Most of these acids, except the sulphonic, will not coat satisfactorily until there is some copper in the solution. For this reason it is preferable to employ a soluble compound of copper to accelerate the action of the solution and the coating is further improved by an oxidizing agent which is compatible with the solution. Any oxidizing agent which does not introduce an objectionable metal or other compound and which does not oxidize the acid used can be employed in suitable proportions. Sodium sulphite, sodium nitrite and sodium nitrate are readily available compounds of this character although, if the nitrate is employed with oxalic acid, the solution should not be heated above the temperature at which the oxalic acid is oxidized. Of course, similar observations apply with other oxidizing agents and other acids of the group described.

There may be considerable variations in the proportions of the acid and other ingredients in the solution, but a proportion which is satisfactory with the group of acids in general is about a 15% solution of the acid with 1% of sodium nitrite and about 1/20 of 1% of copper sulphate. The solutions coat best when hot, but, as observed above, the nature of the oxidizing agent and of the acid being used must be considered in deciding upon the temperature to employ, in order to avoid exhausting the strength of the oxidizing agent and the acid upon each other instead of on the coating operation.

The surface of a copper or copper alloy article dipped in a hot solution of the kind described for ten minutes has formed thereon a substantially integral coating to which paint, varnish or similar siccative coats adhere with great tenacity. The time necessary for the coating will, of course, vary with the strength of the solution, the proportions and nature of the materials used, etc., but the ten minutes mentioned is a fair working time with many typical solutions of this kind.

Apparently the coating formed in the manner described above is essentially a copper salt of the acid employed for the coating operation.

What we claim is:—

1. An article having a surface of copper or copper alloy coated with a substantially integral coating of a salt of copper and acid of the group consisting of dicarboxylic and hydroxydicarboxylic acids of the aliphatic series and carboxylic acids, having one carboxyl group, and sulphonic acids of the aromatic series, and benzene phosphonic acid.

2. The method of coating surfaces of copper or copper alloy, which consists in subjecting the surface to a solution of an acid of the group consisting of dicarboxylic and hydroxydicarboxylic acids of the aliphatic series and carboxylic acids, having one carboxyl group, and sulphonic acids of the aromatic series, and benzene phosphonic acid, said solution containing a soluble compound of copper.

3. The method in accordance with claim 2, and in which the solution contains a compatible oxidizing agent.

4. The method of coating a surface of copper or copper alloy, which consists in subjecting the surface to a solution of oxalic acid, containing a soluble compound of copper and a compatible oxidizing agent.

5. The method of coating a surface of copper or copper alloy, which consists in subjecting the surface to a solution of sulphonic acid of the aromatic series.

ROBERT R. TANNER.  
JOHN S. THOMPSON. 45